# EUROPEAN PATENT SPECIFICATION

(11) **EP 0 588 266 B1**
(45) Date of publication and mention of the grant of the patent: **09.06.1999**
(21) Application number: 93114609.6
(22) Date of filing: 10.09.1993
(51) Int. Cl.: B22D 1/00, B22D 5/00

(54) **Method and apparatus for producing metal objects**
Verfahren und Vorrichtung zur Herstellung von Metallgegenständen
Procédé et appareil pour la fabrication d'objets métalliques

(30) Priority: 14.09.1992 FI 924112
(43) Date of publication of application: 23.03.1994
(73) Proprietor: Outokumpu Wenmec Oy, 02200 Espoo (FI)
(72) Inventor: Majonen, Harri Juhani, SF-02670 Espoo (FI); Marttila, Tom Erland, SF-00210 Helsinki (FI)
(74) Representative: Zipse + Habersack

(56) References cited:
- WO-A-80/02659
- DE-A- 2 316 045
- DE-C- 122 573
- US-A- 4 436 142
- PATENT ABSTRACTS OF JAPAN vol. 6, no. 236 (M-173)(1114) 25 November 1982 & JP-A-57 134 241 (JIDOUSHIYA IMONO K.K.) 19 August 1992

## Description

The present invention relates to a method and apparatus for producing alloy metal objects, advantageously of a standard weight, by means of casting, according to the preamble of claims 1, 5 and 9, respectively. Therein the alloy ingredients are added to the main metal flow after smelting the main metal.

While casting alloy metal objects, the alloy ingredients are usually added, in connection with the smelting of the main metal, to the same smelting furnace in solid state. Prior to the casting, an analysis sample must be taken from the smelting furnace in order to define the right composition, which operation essentially increases the duration of the casting cycle. Moreover, if several alloys containing different alloy ingredients are desired to be cast in the same smelting furnace, the furnace must essentially be completely emptied in order to prevent any mixing of the respective alloys.

DE-A 23 16 045 discloses a method according to the preamble of claim 1. In this device the main metal and alloy metals are added to a mixing furnace, i.e. to melting furnace. The disadvantage of this device is that for each new alloy to be produced the mixing furnace has to be properly cleaned. US-4,436,142 mentions the addition of a nodulizing agent to obtain ductile iron castings. The nodulizing agent causes graphite which is ordinarily present in gray iron castings in flake form to assume a nodular or spheroidal form. A disadvantage of the nodulizing agents is a low-boiling point which leads to serious difficulties which may result in violent pyrotechnic reactions. JP-A-57-134241 discloses an arrangement wherein inoculant material is added to a batched main masse flow between batching member and the molt . However, the addition of materials between the batching member and the mold may lead to inhomogenities in the casted metal mixture.

The object of the present invention is to eliminate some of the drawbacks of the prior art and to achieve an improved and peratively more secure method and apparatus for producing alloy metal objects, essential of a standard weight, by casting so that different alloys can be cast under usage of one smelting furnace without an essential break in the production. The essential novel features of the invention are apparent from the appended patent claims 1, 5 and 9. Advantageous embodiments of the invention are subject matter of the corresponding subclaims.

According to the invention, from the smelting furnace of the main metal, there is conducted molten metal, advantageously at a rate allowed by the smelting capacity of the furnace, to at least one connecting channel provided in between the smelting furnace and the molten metal batching member, which connecting channel can be moved in the transversal and vertical directions. The amount of molten metal to be conducted into the connecting channel is adjusted by means of control members, so that an essentially continuous feeding of molten metal from the smelting furnace into the connecting channel is achieved. The metals to be alloyed, which can be one or several, are conducted in desired quantities to the molten flow in between the smelting furnace and the casting mold, so that the control members adjusting the main metal flow also are advantageously used for adjusting the feeding quantities of the alloy metal or metals, according to the desired alloy ratio and the weight of the metal object to be cast. The alloy metals can be conducted into the main metal flow either in molten or solid state, either into the connecting channel in between the smelting furnace and the molten metal batching member, or directly into the molten metal batching member.

From the connecting channel in between the smelting furnace and the batching member, the molten metal is conducted to the batching member advantageously so, that the connecting channel is shifted vertically downwards by means of shifting members, and the melt begins to flow from the connecting channel to the batching member of the casting mold. Essentially for the duration of the flowing of the melt from the connecting channel to the batching member, the feeding rate of the melt from the smelting furnace to the connecting channel and respectively the feeding rate of the alloy metals to the batching member if can be increased. The feeding of the melt from the connecting channel to the batching member, and the resulting turbulence of the metal alloy, advantageously intensifies the mixing of the metal alloy in an advantageous fashion.

The batching member receives the molten metal flow fed from the connecting channel, and possibly also at least one alloy metal flow fed directly into the batching member. When the same molten metal alloy as in the previous casting cycle is fed into the batching member, a small amount of the said metal alloy is advantageously left in the batching member from the previous casting cycle, so that there can advantageously be taken into account for instance metal losses caused by splashing of the molten metal, as well as metal losses caused by its sticking to the bottom of the batching member. Now a new charge of molten metal, corresponding to the weight of the metal object to be cast, is fed into the batching member. If the metal alloy to be cast should be changed, to the batching member there is fed alloyed molten metal only as much as is necessary in order to make the melt quantity contained in the batching member to correspond to the weight of the metal object to be cast.

When the desired quantity of melt is fed into the batching member, the melt flow into the batching member is stopped, advantageously for instance by lifting the connecting channel and the alloy metal feeding members to their top position. From the batching member, the alloyed melt corresponding in quantity to the object to be cast is conducted into a casting mold by tilting the batching member. Only if the metal alloy to be cast should be changed, the batching member is emptied altogether, otherwise a small amount of the alloyed molten metal to be cast is advantageously left in the batching member as a base charge.

The feeding of the main metal in the metal object to be cast from the smelting furnace to at least one connecting channel in between the smelting furnace and the batching member is advantageously carried out in two successive stages, so that when the connecting channel is in its lifted position, and thus the melt does not flow into the batching member, only molten main metal is fed into the connecting channel. Now the connecting channel advantageously serves as an intermediate tank for the molten main metal, in which case a separate intermediate tank is not needed, and thus one slag-forming transfer of the melt from one tank to another is avoided. On the other hand, when the connecting channel is in its low position, so that the melt flows from the connecting channel to the batching member, the feeding rate of the molten main metal from the smelting furnace into the connecting channel is increased. Essentially simultaneously with the increase of the main metal feeding rate, the feeding of the alloy ingredient or ingredients is switched on, and the alloy ingredients are fed either in solid or molten state to the main metal flow contained in the connecting channel, or directly to the batching member. Thus the main metal flow in the smelting furnace remains clear of the alloy ingredients, and the metal alloy to be cast can be changed simply by changing either the quantity of the alloy ingredient, the alloy ratio or the alloy ingredient, and by feeding the alloy ingredient or ingredients from the smelting furnace to the main metal flow that is already removed from the smelting furnace, in between the smelting furnace and the casting mold. Moreover, the feeding of the alloy ingredient or ingredients to the connecting channel advantageously starts the alloying of the main metal flow already prior to the batching member.

While employing the method and apparatus of the invention for producing metal objects, the alloy ingredient quantity, alloy ratio or alloy ingredient of the metal object can be changed essentially without a break in the production. In similar fashion, each metal object accurately contains a desired amount of alloy metals, and the metal object is essentially accurately of the desired weight. Furthermore, when changing the alloy ingredient quantity, alloy ratio or alloy ingredients, there are not created incorrectly alloyed metal objects, and thus the analysis samples become essentially unnecessary. Moreover, when using the method and apparatus of the invention, the need for space and labour is essentially reduced. Owing to its simplicity, the apparatus requires an essentially small amount of building and installation work in the production facilities, and thus the apparatus is installable essentially rapidly, which increases the applicability of the method and apparatus of the invention.

The invention is explained below with reference to the appended drawing, which represents a preferred embodiment of the invention in a top-view schematical illustration.

According to the drawing, the main metal in the metal object to be alloyed is smelted in the smelting furnace 1. From the smelting furnace 1, the smelted main metal is conducted to the connecting channel 2 advantageously by means of a pump 3, and the molten flow passing therethrough can advantageously be adjusted to be suitable for the capacity of the smelting furnace 1. The quantity of the melt fed into the connecting channel 2 by the pump 3 is adjusted by means of the control member 4. The melt feeding rate is adjusted so that when the connecting channel 2 is in its top position, i.e. during the unloading stage of the batching member 5, the melt feeding rate is advantageously maintained such that only a small amount of melt flows into the chute-like connecting channel 2. On the other hand, when the connecting channel 2 is in its low position, i.e. during the filling stage of the batching members 5, the melt feeding rate is increased, and essentially simultaneously with an increase in the feeding rate, the feeding of alloy ingredients into the connecting channel 2 is begun. One of the alloy ingredients is first smelted in the alloy ingredient smelting furnace 6, and a desired quantity of alloy ingredient per one metal object is conducted via the alloy ingredient batching member 7 to the connecting channel, whereas a desired amount of the second alloy ingredient to be fed in solid state is fed via the alloy ingredient feeder 8 to the molten metal flowing in the connecting channel 2. The feeding of the alloy ingredients to the connecting channel 2 is also advantageously conducted by means of the same control member 4.

From the connecting channel 2, the alloyed molten metal is conducted in batches and in standard charges to the batching member 5. The standard charge essentially corresponds to the weight of the metal object to be cast. In the method of the invention, in the first batching after changing the alloying of the metal object, into the batching member 5 there is, however, fed a batch which corresponds to the weight of the metal object to be cast plus the base charge left in the batching member 5 after unloading the same. This base charge is removed in connection with the last unloading of the batching member 5, which takes place prior to changing the alloying of the metal object.

From the batching member 5, a quantity of the alloyed molten metal corresponding to the weight of the metal object to be cast is discharged into the casting mold 9. There can be several casting molds 9, so that they are located on the same rotating cast line 10. The casting molds 9 can also be located immovably, advantageously in a curved configuration, so that the batching member 5 is located turnably in the center of the circle pertaining to the said curve.

The above specification is a description one preferred embodiment of the invention only, but the invention can be largely modified within the scope of the appended patent claims. For instance, the batching member 5 can advantageously be common for two or several connecting channels 2. Thus even large metal objects can be alloyed with an essentially high accuracy and speed.

## Claims

1. A method for producing a standard-weight metal object, alloyed with at least one alloy ingredient, by means of casting, in which method a batching member (5) is used for feeding the desired amount of melt into the mold (9),
**characterized** in
that the main metal and alloy ingredient flows are controlled so that the main metal is fed into a connecting member (2) between a smelting furnace (1) used for melting the main metal and the batching member (5) in a continuous operation, and that the alloy ingredient is fed into the molten main metal flow between the melting furnace (1) and the batching member (5).

2. A method according to claim 1,
**characterized** in
that the alloy ingredient is fed into the main metal flow in batches.

3. A method according to claim 1 or 2,
**characterized** in
that the alloy ingredient is fed into the main metal flow in molten state.

4. A method according to claim 1 or 2,
**characterized** in
that the alloy ingredient is fed into the main metal flow in solid state.

5. A method for producing a standard-weight metal object alloyed with at least one alloy ingredient by means of casting, in which method a batching member (5) is used for feeding the desired amount of melt into the mold (9),
**characterized** in
that the main metal and alloy ingredient flows are controlled so that the main metal is fed into a connecting member (2) between a smelting furnace (1) used for melting the main metal and the batching member (5) in a continuous operation and that the alloy ingredient is fed into the molten main metal flow in the batching member (5).

6. The method according to claim 5,
**characterized** in
that the alloy ingredient is fed into the main metal flow in batches.

7. The method according to claim 5 or 6,
**characterized** in
that the alloy ingredient is fed into the main metal flow in molten state.

8. The method according to claim 5 or 6,
**characterized** in
that the alloy ingredient is fed into the main metal flow in solid state.

9. An apparatus for realizing the method of claim 1 or 5, comprising a smelting furnace (1) for smelting the main metal, batching members (5) for the alloy ingredient, a connecting channel (2) for transporting the molten metal to be cast, a control member (4) and batching member (5) of the molten metal and a casting mold (9),
**characterized** in
that the connecting channel (2) is installed between the smelting furnace (1) and the batching member (5) to be movable at least vertically with respect to the batching member (5).

10. The apparatus according to claim 9,
**characterized** in
that the connecting channel (2) serves as an intermediate tank for the essentially continuous main metal flow.

11. The apparatus according to one of claims 9 or 10,
**characterized** in
that the number of connecting channels (2) is at least one per each metal object to be cast.

## Patentansprüche

1. Verfahren zur Herstellung eines Metallgegenstandes mit einem Standardgewicht, der mit mindestens einem Legierungsbestandteil legiert wird, mittels Formgießens, in welchem Verfahren eine Dosiervorrichtung (5) zum Zuführen der gewünschten Schmelzmenge in die Gußform (9) verwendet wird,
dadurch gekennzeichnet, daß die Ströme des Grundmetalls und des Legierungsbestandteils gesteuert werden, so daß das Grundmetall einem Verbindungsglied (2) zwischen einem zum Schmelzen des Grundmetalls verwendeten Schmelzofen (1) und der Dosiervorrichtung (5) kontinuierlich zugeführt wird, und daß der Legierungsbestandteil dem geschmolzenen Grundmetallstrom zwischen dem Schmelzofen (1) und der Dosiervorrichtung (5) zugeführt wird.

2. Verfahren nach Anspruch 1,
dadurch gekennzeichnet, daß der Legierungsbestandteil dem Grundmetallstrom chargenweise zugeführt wird.

3. Verfahren nach Anspruch 1 oder 2,
dadurch gekennzeichnet, daß der Legierungsbestandteil dem Grundmetallstrom in geschmolzenem Zustand zugeführt wird.

4. Verfahren nach Anspruch 1 oder 2,
dadurch gekennzeichnet, daß der Legierungsbestandteil dem Grundmetallstrom in festem Zustand zugeführt wird.

5. Verfahren zur Herstellung eines Metallgegenstandes mit einem Standardgewicht, der mit mindestens einem Legierungsbestandteil legiert wird, mittels Formgießens, in welchem Verfahren eine Dosiervorrichtung (5) zum Zuführen der gewünschten Menge an Schmelze in die Gußform (9) verwendet wird,
dadurch gekennzeichnet, daß die Ströme des Grundmetalls und des Legierungsbestandteils gesteuert werden, so daß das Grundmetall einem Anschlußglied (2) zwischen einem zum Schmelzen des Grundmetalls verwendeten Schmelzofen (1) und der Dosiervorrichtung (5) kontinuierlich zugeführt wird, und daß der Legierungsbestandteil dem geschmolzenen Grundmetallstrom in der Dosiervorrichtung (5) zugeführt wird.

6. Verfahren nach Anspruch 5,
dadurch gekennzeichnet, daß der Legierungsbestandteil dem Grundmetallstrom chargenweise zugeführt wird.

7. Verfahren nach Anspruch 5 oder 6,
dadurch gekennzeichnet, daß der Legierungsbestandteil dem Grundmetallstrom in geschmolzenem Zustand zugeführt wird.

8. Verfahren nach Anspruch 5 oder 6,
dadurch gekennzeichnet, daß der Legierungsbestandteil dem Grundmetallstrom in festem Zustand zugeführt wird.

9. Vorrichtung zur Ausführung des Verfahrens von Anspruch 1 oder 5, umfassend einen Schmelzofen (1) zum Schmelzen des Grundmetalls, Dosiervorrichtungen (5) für den Legierungsbestandteil, einen Verbindungskanal (2) zum Transportieren des zu gießenden geschmolzenen Metalls, ein Steuerglied (4) und eine Dosiervorrichtung (5) für das geschmolzene Metall und eine Gußform (9),
dadurch gekennzeichnet, daß der Verbindungskanal (2) zwischen dem Schmelzofen (1) und der Dosiervorrichtung (5) derart angeordnet ist, daß er bezüglich der Dosiervorrichtung (5) zumindest vertikal verschiebbar ist.

10. Vorrichtung nach Anspruch 9,
dadurch gekennzeichnet, daß der Verbindungskanal (2) ein Zwischenbehälter für den im wesentlichen kontinuierlichen Grundmetallstrom dient.

11. Vorrichtung nach Anspruch 9 oder 10,
dadurch gekennzeichnet, daß zumindest ein Verbindungskanal (2) für jeden zu gießenden Gegenstand vorgegeben ist.

## Revendications

1. Procédé de fabrication d'un objet métallique de poids standard, allié avec au moins un ingrédient d'alliage, par coulée, un élément de dosage (5) étant utilisé dans ce procédé pour distribuer la quantité désirée de métal fondu dans le moule (9),
caractérisé en ce que :
les écoulements de métal principal et d'ingrédient d'alliage sont réglés de sorte que le métal principal est introduit dans un élément de liaison (2) entre un four de fusion (1), utilisé pour la fusion du métal principal, et l'élément de dosage (5) en une opération continue, et
l'ingrédient d'alliage est introduit dans l'écoulement de métal principal fondu entre le four de fusion (1) et l'élément de dosage (5).

2. Procédé selon la revendication 1, caractérisé en ce que l'ingrédient d'alliage est introduit par cuvées dans l'écoulement de métal principal.

3. Procédé selon la revendication 1 ou 2, caractérisé en ce que l'ingrédient d'alliage est introduit dans l'écoulement de métal principal à l'état fondu.

4. Procédé selon la revendication 1 ou 2, caractérisé en ce que l'ingrédient d'alliage est introduit dans l'écoulement de métal principal à l'état solide.

5. Procédé de fabrication d'un objet métallique de poids standard allié avec au moins un ingrédient d'alliage par coulée, un élément de dosage (5) étant utilisé dans ce procédé pour distribuer la quantité désirée de métal fondu dans le moule (9),
caractérisé en ce que :
les écoulements de métal principal et d'ingrédient d'alliage sont réglés de sorte que le métal principal est amené dans un élément de liaison (2) disposé entre un four de fusion (1) utilisé pour fondre le métal principal et l'élément de dosage (5) en une opération continue, et
l'ingrédient d'alliage est introduit dans l'écoulement de métal principal fondu dans l'élément de dosage (5).

6. Procédé selon la revendication 5,
caractérisé en ce que l'ingrédient d'alliage est introduit dans l'écoulement de métal principal, en cuvées.

7. Procédé selon la revendication 5 ou 6, caractérisé en ce que l'ingrédient d'alliage est introduit à l'état fondu dans l'écoulement de métal principal.

8. Procédé selon la revendication 5 ou 6, caractérisé en ce que l'ingrédient d'alliage est introduit à l'état solide dans l'écoulement de métal principal.

9. Appareil pour la mise en oeuvre du procédé de la revendication 1 ou 5, comprenant un four de fusion (1) pour fondre le métal principal, des éléments de dosage (7) pour l'ingrédient d'alliage, un canal de liaison (2) pour transporter le métal fondu à couler, un élément de réglage (4) et un élément de dosage (5) du métal fondu et un moule de coulée (9),
caractérisé en ce que le canal de liaison (2) est installé entre le four de fusion (1) et l'élément de dosage (5) de manière à être déplaçable au moins verticalement par rapport à l'élément de dosage (5).

10. Appareil selon la revendication 9, caractérisé en ce que le canal de liaison (2) sert de réservoir intermédiaire pour l'écoulement sensiblement continu du métal principal.

11. Appareil selon une des revendications 9 ou 10,
caractérisé en ce que le nombre de canaux de liaison (2) est au moins d'un pour chaque objet métallique à couler.
